

## UNITED STATES PATENT OFFICE

2,316,379

PROCESS OF REMOVING IMPURITIES FROM  
WASHED TEXTILES

Erhart Wolter, Dusseldorf-Benrath, Germany,  
assignor, by mesne assignments, to The Pro-  
cter & Gamble Company, Cincinnati, Ohio, a  
corporation of Ohio

No Drawing. Application June 24, 1939, Serial  
No. 280,916. In Germany June 28, 1938

2 Claims. (Cl. 252—143)

This invention relates to a process for removing water insoluble soaps or precipitates from textiles which have been treated with those washing agents which form insoluble precipitates in hard water.

When textiles are cleansed in hard water, most washing agents leave a water-insoluble precipitate which prevents thorough cleansing and dulls the fibers. These precipitates, in some instances, may even cause permanent damage if they are not thoroughly removed. Various partially successful methods have been advanced for removing these precipitates. One of these methods involves the use of dilute solutions of acids, such as baths containing acetic acid.

Crystallized acids have proved especially advantageous for household use because they occupy less space, are more easily stored and handled and are much more easily dosed than dilute acid solutions of varying concentration. Oxalic acid in crystalline form has been used for this purpose.

It is an object of this invention to provide a highly effective method for removing detrimental water-insoluble precipitates from textiles involving the use of an inexpensive, readily available acid treating agent.

In accordance with this invention, treatment baths acidulated with amidosulfonic acid or sulfamic acid have proven surprisingly effective in removing detrimental water-insoluble precipitates deposited upon textiles in washing operations. Sulfamic acid is easy to prepare, inexpensive, is readily available and may be used in the crystalline state or in aqueous solutions.

In the preparation of rinsing baths, the sulfamic acid is preferably introduced as crystals either alone or in combination with inert water-soluble materials, such as salts. Since the acid is stable in aqueous solutions, it may be marketed in such solutions for introduction into rinsing baths without a material loss in effectiveness.

The relative efficiency of the instant acid compound as compared with compounds of the prior art may quickly be observed from the tests set out below, wherein the effectiveness of the dif-

ferent agents may be judged from the ash content of several different types of washed fabrics. The degree of effectiveness of acetic, oxalic and sulfamic acids in concentrations of five grams of acid per liter of treatment liquid when treating linens, mixed fabrics and chiffons for a quarter of an hour to remove detrimental deposits is made clear.

|              | Percent ash after washing only | Percent ash after treatment with acetic acid | Percent ash after treatment with oxalic acid | Percent ash after treatment with amido-sulfonic acid |
|--------------|--------------------------------|----------------------------------------------|----------------------------------------------|------------------------------------------------------|
| 15 Linen     | 7.3                            | 4.3                                          | 2.1                                          | 0.17                                                 |
| Mixed fibers | 10.3                           | 7.5                                          | 2.3                                          | 0.12                                                 |
| Chiffon      | 11.3                           | 7.0                                          | 2.6                                          | 0.33                                                 |

The foregoing results clearly show the superiority of the processes and treatment baths for removing detrimental deposits resulting from washing operations when acidulation is produced through the use of sulfamic acid.

The amount of sulfamic acid required is not critical and may be varied in relation to the quantity of the deposits or hardness of the water. Under one percent in the rinsing bath is sufficient.

It should be understood that the present invention is not limited to the specific compositions and processes herein set out, but that its scope is to be judged by the wording of the appended claims as interpreted in the light of the general tenor of the specification.

35 I claim:

1. The method of removing deleterious deposits from a textile material washed in hard water, which comprises rinsing said material in an aqueous rinsing bath acidulated with approximately .5% sulfamic acid.

2. The method of removing deleterious deposits from textile materials washed in hard water, which comprises rinsing said materials in a rinsing bath comprising water and less than 1% sulfamic acid.

ERHART WOLTER.